

# United States Patent Office

2,777,255

Patented Jan. 15, 1957

1

2,777,255

## METHOD FOR PRODUCING IMPROVED MONOCRYSTALLINE REFRACTIVE MATERIAL

Leon Merker, New York, N. Y., assignor to National Lead Company, New York, N. Y., a corporation of New Jersey

No Drawing. Application February 2, 1953,  
Serial No. 334,709

1 Claim. (Cl. 49—89)

This invention relates to monocrystalline strontium titanate and to methods of making and treating monocrystalline strontium titanate.

Monocrystalline strontium titanate is characterized by a high index of refraction (about 2.4) and a low reciprocal relative dispersion or  $v$  value (about 13). Large single crystals of strontium titanate may be made which are clear, transparent and glass-like and such crystals have important optical applications because the index is substantially higher and the reciprocal relative dispersion substantially lower than those of the densest flint glasses. Whether clear or colored, the crystals have important gem stone and other applications because of their high refraction and dispersion.

One broad use of optical materials having high refractive indices and high dispersion is in the manufacture of lenses and prisms. For example, materials having a high index of refraction are utilized in the construction of optical systems such as telescopic or high magnification microscopic objectives. Furthermore combinations of optical materials which individually possess widely variant optical properties are used to prepare achromatic lenses. High dispersion qualities are also useful for making prisms and the like. Highly refractive single crystal material is also useful for the preparation of ornamental objects such as gem stones. Synthetic gems of various types and colors are in great demand for both personal adornment and industrial uses.

An object of this invention therefore is to provide a method for producing a monocrystalline material which possesses exceedingly high index of refraction with a high dispersion or relatively low  $v$  value. A further object is to provide a method for producing monocrystalline glass-like material suitable for manufacture of lenses, prisms, gem stones, and the like which is clear and substantially transparent and which possesses a substantially white color. Further to provide a process for producing a clear and transparent single crystal of glass-like material substantially free from internal strains from a single crystal boule which possesses a substantially black color. These and other objects will become apparent from the following more complete description of the instant invention.

Broadly this invention contemplates a process for producing an improved single crystal of strontium titanate which comprises annealing the single crystal of strontium titanate in an oxidizing atmosphere at a high temperature to relieve the strains therefrom and then subjecting the annealed crystal to an oxidizing atmosphere at temperature of about 200° C. to about 500° C. to improve the color. It has been found that the internal strains in the single crystal strontium titanate may be relieved by annealing the crystal in an oxidizing atmosphere at temperature from about 1000° C. to about 1700° C. for 12 to 180 hours. The color of the annealed crystal may be improved by subsequently treating the crystal in an oxidizing atmosphere at temperature from about 200° C. to about 500° C. for 6 hours to 80 hours.

Copending application Serial No. 252,906 filed October

24, 1951, now U. S. Patent No. 2,628,156, filed by Leon Merker and Langtry E. Lynd describes and claims in general a monocrystalline mass of strontium titanate. The instant invention covers a method for more properly annealing the monocrystalline strontium titanate boule to obtain a substantially strain-free white boule. Copending application Serial No. 252,906 is assigned to the same assignee as the instant invention.

The term strontium titanate is intended to embrace both pure and substantially pure  $\text{SrTiO}_3$ , the latter which contains impurities or added coloring or modifying agents either present or added which are of a nature and in amount so as to not affect the monocrystalline structure nor alter the desired color of the strontium titanate material produced. In most cases the impurities are held to a minimum and ordinarily will not exceed a few tenths of a percent and modifying or coloring agents are added in the amount necessary to produce the desired effect.

In order to prepare a monocrystalline mass by co-fusing particles of strontium titanate, it is necessary to employ high temperatures. Strontium titanate melts in the neighborhood of about 2050° C. and it is therefore preferred to use an oxygen-hydrogen flame in order to obtain the necessary temperatures without the possible introduction of impurities.

It is convenient to drop finely divided strontium titanate particles into the area of intense heat formed by the oxygen-hydrogen flame, i. e. in or near the oxygen cone. Within this area the strontium titanate melts and when carefully cooled builds up as a single crystal on a base which holds the molten strontium titanate material.

In order to start such a single crystal to form it is desirable to first form a seed and then gradually build up the amount of molten material on the seed to form the crystal. Such a procedure allows the crystal to build up upon itself gradually increasing in diameter until a boule or carrot-shaped single crystal of strontium titanate is formed.

It is preferred to employ a strontium titanate powdered material which is substantially free from objectionable or incompatible impurities which detrimentally would affect the crystal structure. Starting material should be finely divided and fairly uniform in size. Such a material may be conveniently prepared by first reacting titanium oxalate with strontium chloride to precipitate strontium titanium oxalate. After thoroughly washing the strontium titanium oxalate, it is heated at a temperature of at least 500° C. to remove the oxalate portion thus forming strontium titanate. Preferably this strontium titanate material is then crushed and ground to obtain finely divided material from which the strontium titanate single crystal is subsequently formed.

Using an oxygen-hydrogen burner and passing the finely divided strontium titanate feed material into the intensely heated zone, a single crystal boule of strontium titanate 1 inch long and  $\frac{1}{2}$  inch wide was prepared in 2 hours.

In order to produce an improved type of strontium titanate single crystal, the black boule was subjected to the oxidation treatment contemplated in the instant invention. The black boule was treated at temperature of 1500° C. for 25 hours and was then cooled slowly to 300° C. temperature and held at 300° C. temperature for 48 hours. The boule after treatment possessed a substantially transparent appearance with a substantially white color. It was also free from strains. According to the process of the instant invention, in order to produce a superior type of boule which is substantially free from strains, it is necessary to employ the above-described double oxidation treatment.

The single crystal material should be subjected first to a very high temperature oxidation treatment, i. e. from

## 3

temperatures of about 1000° C. to about 1700° C. These high temperature treatments should be maintained between 12 and 180 hours. At this stage the monocrystalline strontium titanate possesses a purplish or pinkish appearance instead of the former black color. The monocrystalline material is then subjected to the second oxidation treatment which should be carried out at temperature from about 200° C. to about 500° C. for 6 hours to 80 hours. This low temperature treatment is necessary in order to obtain a substantially white boule. The two oxidation treatments can be carried out in separate furnaces or in the same furnace by merely lowering the temperature after the first treatment to that required for the second. When the monocrystalline strontium titanate material is processed according to the instant invention the strains in the crystal are relieved and boules which are properly annealed are obtained. These monocrystalline masses of strontium titanate are substantially white in color and are properly annealed and may be shaped into many bodies useful for optical purposes such as, e. g. 20 cut into lens blanks suitable for preparation of lenses, prisms, and other optical products; and also may be cut into various shapes and sizes to produce many articles such as ornamental objects and novelty gems, which depend for their attractiveness and usefulness on the high refractive index of the material of which they are composed.

The index of refraction of the strontium titanate crystal is extremely high, i. e. about 2.4, and the reciprocal dispersion is about 13. These values will vary slightly as various types of starting materials and processing conditions are employed.

It should be noted that the strontium titanate crystal when cut into a lens has a high magnifying power and a short focal length. Such material is particularly useful for telescopic and microscopic objectives and the like, for achromatic lenses and prisms and for other optical purposes which advantageously utilize wide fields, high apertures and short focal lengths. It should be noted that 35 the index of refraction and reciprocal dispersion are very different from any type of known glass.

This monocrystalline mass of strontium titanate after

proper annealing according to this invention will not tend to chip, splinter or crack as easily as those crystals which are not properly annealed.

While this invention has been described and illustrated by the examples shown, it is not intended to be strictly limited thereto and other modifications and variations may be employed within the scope of the following claim.

I claim:

Method for producing an improved single crystal of strontium titanate prepared by co-fusion of finely divided strontium titanate particles which comprises annealing the single crystal of strontium titanate in an oxidizing atmosphere at temperatures from about 1000° C. to about 1700° C. for 12 to 180 hours to relieve the strains in said crystal and subsequently heating the crystal in an oxidizing atmosphere at temperatures from about 200° C. to about 500° C. for 6 to 80 hours to improve the color.

## References Cited in the file of this patent

## UNITED STATES PATENTS

|           |                 |                |
|-----------|-----------------|----------------|
| 988,230   | Verneuil        | Mar. 28, 1911  |
| 1,004,505 | Verneuil        | Sept. 26, 1911 |
| 1,298,540 | Miller          | Mar. 25, 1919  |
| 1,436,164 | Goldschmidt     | Nov. 21, 1922  |
| 2,507,253 | Howatt          | May 9, 1950    |
| 2,610,129 | Eversole et al. | Sept. 9, 1952  |
| 2,628,156 | Merker et al.   | Feb. 10, 1953  |
| 2,634,554 | Barnes          | Apr. 14, 1953  |

## FOREIGN PATENTS

|         |               |                |
|---------|---------------|----------------|
| 243,251 | Great Britain | Nov. 26, 1925  |
| 252,698 | Switzerland   | Oct. 1, 1948   |
| 608,453 | Great Britain | Sept. 15, 1948 |
| 662,782 | France        | Nov. 26, 1927  |
| 664,889 | Great Britain | Jan. 16, 1952  |

## OTHER REFERENCES

"G. E. C. Journal," August 1944, pages 56-59.  
Kremers: "Synthetic Optical Crystals," Ind. and Eng. Chem., November 1940, vol. 32, pages 1478-1482.